

June 8, 1965

C. R. MORELOCK  
USE OF THE WORKING MATERIAL AS PART OF  
THE CRYSTAL MAKING APPARATUS  
Filed May 31, 1962

3,188,182



Inventor:  
Charles R. Morelock,

by *Richard R. Speer*  
His Attorney.

1

3,188,182

**USE OF THE WORKING MATERIAL AS PART OF  
THE CRYSTAL MAKING APPARATUS**Charles R. Morelock, Ballston Spa, N.Y., assignor to  
General Electric Company, a corporation of New  
York

Filed May 31, 1962, Ser. No. 200,023

3 Claims. (Cl. 23—273)

This application is a continuation-in-part of applicant's copending application, Serial No. 120,560, filed June 29, 1961, now abandoned, and assigned to the same assignee as the present invention.

This invention relates to metal single crystals and more particularly to improved processes and apparatus for producing such crystals.

Prior to this invention, the production of vapor-deposited single crystals has been limited to those materials having low melting points and relatively high oxide dissociation pressures. The greatly improved physical properties offered by single crystals, as compared to polycrystalline materials, have not been attainable due to the absence of processes for effectively producing such crystals.

It is a principal object of this invention to provide an improved process for producing metal single crystals or whiskers.

Another object of this invention is to provide an improved process for producing single crystals of metals having low oxide dissociation pressures.

An additional object of this invention is to provide improved apparatus for producing metal single crystals.

Other objects and advantages of the present invention will be in part obvious and in part explained by reference to the accompanying specification and drawings.

In the drawings:

FIG. 1 is a side elevation, partly in section, showing an apparatus for producing metal crystals according to the present invention;

FIG. 2 is a perspective showing a combined source metal and substrate growth body for use in the apparatus of FIG. 1;

FIG. 3 is a perspective of another form of source metal-growth substrate combination; and

FIG. 4 is yet another form of source metal and growth substrate combination for growing single crystals.

The process of this invention generally comprises locating a source metal body, which may be made of a metal such as chromium, copper, gold, nickel, iron, cobalt, or binary or ternary alloys of iron, nickel and cobalt in a chamber isolated from the outside atmosphere, which chamber can be heated to a temperature sufficient to vaporize the source metal. A growth substrate body which may be compositionally identical to the source metal, or of a different composition if desired, is also located within the vaporizing chamber that is maintained at a temperature lower than that of the source metal body. As the chamber is heated to a temperature sufficient to vaporize the source metal, the chamber is continuously evacuated so that some portion of the source metal vapor in the chamber escapes toward the outlet and getters oxygen from the chamber to maintain the oxygen pressure therein below the dissociation pressure of the source metal oxide.

The apparatus of this invention generally comprises means defining a vaporizing chamber, such as a fused silica tube, evacuating means operably connected to the vaporizing chamber so that the atmosphere within the chamber can be continuously removed, a body of source metal and a growth substrate body located within the

2

vaporizing chamber, and means to maintain the temperature of the growth substrate body below that of the source metal body.

The apparatus of the invention can be described more completely by referring to FIG. 1 of the drawings. In this figure, the numeral 10 indicates the vaporizing chamber, this chamber being defined by a fused silica tube 11 and surrounded by heating means, here shown as a platinum-wound furnace 12. The furnace 12 surrounds only a portion of the entire length of tube 11 so that the heating zone where vaporization and deposition of metal single crystals is carried out is not coextensive with the entire length of tube 11. A Pyrex tube 15 has been integrally joined to the upper end of tube 11 and the upper end of this tube is connected to a source of vacuum, not shown. Extending outwardly from but integrally joined to the tube 15 is a lateral extension 16 which is completely sealed so that no opening is present into the volume defined by tubes 11 and 15. The Pyrex glass was substituted for quartz in the manner described because it is easier to work and shape and is cheaper in the overall construction of the apparatus.

A generally cylindrical source metal body 20 is shown positioned within the hot zone of vaporizing chamber 10, the body 20 having, of course, an axial opening extending through it. A growth substrate body is located approximately equidistant from the inner surface of body 20 and extends upwardly beyond the upper limit of body 20 a distance sufficient to permit a portion of its length to be located outside of the hot zone defined by furnace 12.

The growth substrate body 21 can be lowered into the operating position shown and, conversely, raised completely out of the hot zone defined by furnace 12 by means of the winch mechanism indicated generally by numeral

35 25. This mechanism comprises a tungsten wire 26 which can be wound and unwound onto reel 27. The reel 27 is fixedly attached to rotatable shaft 28 mounted in journal 29. That end of shaft 28 furthest removed from reel 27 has a magnet 30 connected to it, which magnet

40 40 can be operated by the rotatable operating member 31. Member 31 comprises a body portion 32 constructed of any suitable plastic or non-conducting material and contains a plurality of magnets 33 which cooperate with the magnet 30 to rotate shaft 28 as member 31 is turned.

45 45 As shown in the figure, clockwise rotation of member 31 will wind fiber 26 on reel 27 and raise substrate body 21 out of operating position within the vaporizing chamber 10.

Generally speaking, when the various elements of the 50 50 apparatus are in the positions indicated in FIG. 1, metal single crystals, or whiskers, can be grown by operating furnace 12 to raise the temperature within vaporizing chamber 10 to a point sufficient to effect vaporization of the source metal body 20. Since a portion of the growth substrate body 21 is isolated from direct radiation by furnace 12, the source metal itself in fact creating this isolation, the temperature of that portion of the growth substrate body located within body 20 will be lower than that of the source metal. Additionally, heat is conducted 55 60 upwardly along the length of body 21 and some proportion radiated outwardly from that portion of body 21 which is located beyond the limits of the hot zone defined by furnace 12. Thus, metal vapor present in chamber 10 will deposit as single crystals.

It is felt that the single crystals or whiskers nucleate on emergent screw dislocations located on or in the surface of the substrate body. Once started by this initial nucleation, the screw dislocation becomes built into the crystal and axial growth proceeds by metal atoms being

adsorbed on the sides of the crystal, migrating to the tip, and becoming incorporated in the lattice at the step of the screw dislocation.

According to this mechanism, crystals should grow at supersaturation ratios which are less than some critical supersaturation ratio,  $\alpha^*$ , required for measurable two-dimensional homogenous nucleation. The supersaturation ratio,  $\alpha$ , is equal to  $p/p_0$ , where  $p$  is the actual pressure of the depositing vapor and  $p_0$  the saturation pressure of the deposited vapor. These pressures are established by the temperatures of the evaporation and growth substrate surfaces.

According to the proposed growth mechanism, there should be no lower vapor pressure limit for the occurrence of single crystal growth. For the metals with which this invention is particularly concerned, viz., chromium, copper, gold, nickel, iron, cobalt, or binary or ternary alloys of iron, nickel and cobalt, no single crystals were grown at vapor pressures less than  $10^{-6}$  mm. of mercury. It is probable that the gettering action of the metal vapor, made possible by continuous evacuation of the vaporizing chamber, is sufficient to keep the oxygen pressure in the growth zone below the dissociation pressure of the metal oxide only at metal vapor pressures of  $10^{-6}$  or greater. The dissociation pressures for the oxides of chromium, iron, cobalt, nickel and copper are approximately  $10^{-20}$ ,  $10^{-12}$ ,  $10^{-10}$ ,  $10^{-8}$ , and  $10^{-7}$  mm. of mercury, respectively. Since in all the experiments conducted the metal vapor pressures were all nearly the same, it would be expected that oxides in the chromium experiments would be more severe than the copper experiments. This was observed to be true.

It is therefore important in carrying out the present process that before the condition of saturation ratio is established, the partial pressure of oxygen must be below the dissociation pressure of the particular metal oxide if whisker growth is to occur. The upper vapor pressure limit should only be  $p_0$  at the melting point,  $T_m$ , of the metal being investigated. The closest approach to this limitation has been in experiments with gold and copper, whiskers having been grown when the substrate temperature was held within  $20^\circ$  C. of their respective melting points.

Whisker growths, then, are not restricted to any particular magnitude of the metal vapor pressures but rather to the upper and lower limits determined as above. This is substantiated by the fact that the vapor pressures used in whisker growth investigations have ranged from  $10^{-7}$  mm. of mercury for gold, to 0.1 mm. of mercury for cadmium.

Several experiments were run to grow metal single crystals or whiskers of various types of metals. In these experiments, growth substrate bodies and source metal bodies were positioned in the vaporizing chamber as shown in FIG. 1 of the drawings while the chamber was being heated continuously by furnace 12 and was also being continuously evacuated. In these experiments, the apparatus was heated to operating temperature prior to the lowering of the growth substrate body into the vaporizing chamber so that any oxygen or other atmospheric contaminants in the apparatus were removed as low as possible. The useful ranges of the evaporation temperatures for the various materials are listed in the following Table I.

Table I

| Metal:   | Evaporation temperature Range, $^\circ$ C. |
|----------|--------------------------------------------|
| Chromium | 830-1890                                   |
| Nickel   | 1080-1455                                  |
| Gold     | 700-1063                                   |
| Copper   | 820-1083                                   |
| Iron     | 1050-1539                                  |
| Cobalt   | 1000-1495                                  |

The source metal, evaporation temperature, growth time, whisker length and the composition of the growth substrate for these various samples are all listed in Table II following:

5

Table II

|    | Evap. Metal       | Evap. Temp. ( $^\circ$ C.) | Growth Time (Hrs.) | Longest Whiskers ( $\mu$ ) | Growth Substrate |
|----|-------------------|----------------------------|--------------------|----------------------------|------------------|
| 10 | CR                | 1,050                      | 16                 | 70                         | Mo Screen.       |
|    | CR                | 900                        | 50                 | None                       | Do.              |
|    | Ni                | 1,200                      | 16                 | 100                        | Do.              |
|    | Ni                | 1,050                      | 48                 | None                       | Do.              |
|    | Au                | 1,050                      | 16                 | 300                        | Au Sheet.        |
|    | Au                | 875                        | 120                | 150                        | Do.              |
|    | Cu                | 830                        | 70                 | None                       | Cu Sheet.        |
| 15 | Cu                | 930                        | 16                 | 200                        | Do.              |
|    | Cu                | 1,020                      | 1                  | None                       | Do.              |
|    | Cu                | 1,000                      | 3                  | 100                        | Do.              |
|    | Cu                | 1,000                      | 16                 | 100                        | Do.              |
|    | Cu                | 950                        | 50                 | 300                        | Do.              |
|    | Fe                | 1,030                      | 16                 | None                       | Fe Sheet.        |
|    | Fe                | 1,060                      | 16                 | 200                        | Do.              |
| 20 | Fe                | 1,150                      | ½                  | None                       | Mo Screen.       |
|    | Fe                | 1,150                      | 1                  | 15                         | Do.              |
|    | Fe                | 1,050                      | 50                 | 200                        | Fe Sheet.        |
|    | Fe                | 1,150                      | 16                 | 100                        | Do.              |
|    | Co                | 1,020                      | ½                  | 5                          | Mo Sheet.        |
|    | Co (23%)-Fe (77%) | 1,120                      | ½                  | 50                         | Do.              |

25 As mentioned previously, it is necessary that the growth substrate body be maintained at a temperature below that of the source metal body if crystal growth is to be obtained. This temperature differential can be obtained in any one of several different ways. For example, in FIG.

30 2 of the drawings, the growth substrate body and source metal body exist as a single unit, here shown as a spirally-wound coil 35. In this case, metal is evaporated from the inner surface of the outermost spiral of coil 35, since it is subjected directly to radiant heating from the furnace

35 and deposited on the outermost surface of the second spiral 37 since this surface is protected from direct heating of the furnace and is therefore somewhat cooler. This same vaporizing and depositing process takes place on each successive spiral, progressing inwardly and ending

40 at the innermost spiral 38. It has been found that the normal temperature differential existing between successive spirals is about  $17^\circ$  C., temperature differentials on the order of  $15^\circ$  and more normally being sufficient to deposit vaporized metal for whisker growth.

45 A slightly modified combined form of source metal body and growth substrate body is indicated by numeral 40 in FIG. 3 of the drawings. In this case, the source metal is a flat sheet 41 which is connected to a larger growth substrate body 42 by means of connecting pieces

50 43. The body 42 is somewhat longer than body 41 so that it can extend upwardly out of the hot zone defined by the heating furnace in much the same manner as the growth substrate body 21 shown in FIG. 1 of the drawings. Although in this case the growth body 42 is subjected to direct heating by the surrounding furnace, not shown, it is of much larger cross section so that the heat will be conducted upwardly into and dissipated from that portion located outside of the hot zone. By utilizing this geometry, it is possible to maintain a sufficient temperature differential between bodies 41 and 42 to deposit crystals on the substrate 42.

55 FIG. 4 of the drawings illustrates a particular form of source metal body-growth substrate body combination which is particularly useful in the present invention.

60 65 In this instance, the source metal body is shown as a wire 50 which extends down through the center of a completely closed growth substrate body 51. The wire 50 is insulated from body 51 by means of an insulating grommet 52 but is electrically connected to the bottom plate of body 51 so that electricity can be made to flow through both body 50 and body 51. The electricity is supplied from a source 53 via the wires 54. The operation of this device is effected by placing the structure in the vaporizing zone, such as shown in FIG. 1, and heating the assembly to a temperature below that where any metal

condensation will occur. By then conducting a flow of electricity through the two bodies, the temperature of wire 50 can be raised beyond the temperature of body 51. This temperature differential results from the carrying capacity of the two bodies. That is, the relatively small size of wire 50 results in a resistance greater to the passage of electricity than is present in body 51, so that electrical heating of wire 50 is effected beyond that which takes place in body 51. This apparatus makes it possible to accurately control the temperature differential between the growth substrate body and the source metal body.

The function of continuously evacuating the vaporizing chamber is important to this invention. Since metals having extremely low oxide dissociation pressures are contemplated, it is necessary that any oxygen in the system be removed to a level as low as possible. It is further essential that oxygen diffusing into the system through the walls of the various vessels be prevented from coming into contact with metal vapor in the growth zone. These objectives are attended by continuously evacuating the atmosphere from vaporizing zone 10 in a manner such that a continuous supply of metal vapor is directed upwardly through tubes 11 and 15 to getter out any oxygen which may be present. This operation makes it possible for the first time to maintain the oxygen pressure in the vaporizing chamber below the dissociation pressure of the source metal oxides, where the metals being vaporized are extremely strong oxide formers. Of course, the apparatus and process are equally effective in growing crystals of those materials where oxygen contamination is a relatively minor problem.

Although the present invention has been described in connection with preferred embodiments, it is to be understood that modifications and variations may be resorted to without departing from the spirit and scope of the invention, as those skilled in the art will readily understand. Such modifications and variations are considered to be within the purview and scope of the invention and the appended claims.

What I claim as new and desire to secure by Letters Patent of the United States is:

1. An apparatus for growing metal single crystals comprising, means defining a vaporizing chamber for growing single crystals of a source metal on a substrate, means operably connected to said vaporizing chamber to effect continuous evacuation of the atmosphere therefrom during operation, means for heating said source metal body and said substrate body, and means separate from said

heating means for rendering the temperature of said substrate body below that of said source metal body, said separate means being in part said source metal body.

2. An apparatus for growing metal single crystals comprising, means defining a vaporizing chamber for growing single crystals of a source metal on a substrate, means operatively connected to said vaporizing chamber to effect continuous evacuation of the atmosphere therefrom during operation, means for heating said source metal body and said substrate body, means separate from said heating means for rendering the temperature of said substrate body below that of said source metal body, and means electrically connecting said source metal body and said substrate body to a source of electricity to provide for a flow of electricity through said bodies, to render the temperature of said substrate body below that of said source metal body.

3. An apparatus as defined in claim 1 wherein said substrate body includes a portion extending beyond the hot zone created by said heating means to withdraw heat from a portion located within the hot zone and thereby maintain the portion within the hot zone at a temperature lower than that of said source metal body.

25

#### References Cited by the Examiner

##### UNITED STATES PATENTS

|           |       |                 |         |
|-----------|-------|-----------------|---------|
| 1,601,931 | 10/26 | Van Arkel       | 148—1.6 |
| 1,617,161 | 2/27  | Hoffman         | 148—1.6 |
| 2,754,259 | 7/56  | Robinson et al. | 148—1.6 |
| 2,813,811 | 11/57 | Sears           | 148—1.6 |
| 2,836,524 | 5/58  | Brenner et al.  | 148—1.6 |
| 2,842,468 | 7/58  | Brenner         | 148—1.6 |
| 2,842,469 | 7/58  | Fullman et al.  | 148—1.6 |
| 2,895,858 | 7/59  | Sangster        | 148—1.6 |
| 3,060,013 | 10/62 | Harvey          | 48—1.6  |

##### FOREIGN PATENTS

|         |       |                |
|---------|-------|----------------|
| 802,842 | 10/58 | Great Britain. |
| 853,979 | 11/60 | Great Britain. |

##### OTHER REFERENCES

- Griest et al., article in the Journal of Applied Physics, vol. 27, September 1956, pages 1022—1024.  
 45 Holland, Vacuum Deposition of Thin Films, John Wiley and Sons, Inc., 1956, page 20.

DAVID L. RECK, Primary Examiner.